# EUROPEAN PATENT SPECIFICATION

(11) **EP 2 997 168 B1**
(45) Date of publication and mention of the grant of the patent: **03.03.2021**
(21) Application number: 14734592.0
(22) Date of filing: 16.05.2014
(51) Int. Cl.: C21D 8/02, C22C 38/34, C22C 38/32, C22C 38/26, C22C 38/22, C22C 38/06, C21D 1/18, C22C 38/18, C22C 38/12, C22C 38/04, C22C 38/02, C22C 38/00, C23C 2/06, C23C 2/02, C21D 9/46, C22C 38/38, C21D 1/78, C21D 6/00, C23C 2/40

(54) **METHOD FOR PRODUCING A HOT DIP GALVANIZED AND OR GALVANNEALED STEEL SHEET BY QUENCHING AND PARTITIONING**
VERFAHREN ZUM HERSTELLEN EINES FEUERVERZINKTEN UND WÄRMEBEHANDELTEN STAHLBLECHES DURCH ABSCHRECKEN UND PARTITIONIEREN
PROCÉDÉ DE FABRICATION D'UNE TÔLE D'ACIER GALVANISÉE ET OU GALVANNEE PAR IMMERSION À CHAUD, PAR TRANCHÉ ET PARTITIONNEMENT

(30) Priority: 17.05.2013 US 201361824699 P; 17.05.2013 US 201361824643 P
(43) Date of publication of application: 23.03.2016
(73) Proprietor: Ak Steel Properties, Inc., West Chester, OH 45069 (US)
(72) Inventor: THOMAS, Grant, Aaron, Liberty Township, OH 45011 (US); LOSZ, Jose Mauro, B., Middletown, OH 45042 (US)
(74) Representative: Samson & Partner Patentanwälte mbB
(86) International application number: PCT/US2014/038364
(87) International publication number: WO 2014/186689

(56) References cited:
- EP-A1- 2 325 346
- EP-A1- 2 524 970
- WO-A1-2005/108058
- WO-A1-2009/035576
- JOHN G SPEER ET AL: "Analysis of Microstructure Evolution in Quenching and Partitioning Automotive Sheet Steel", METALLURGICAL AND MATERIALS TRANSACTIONS A, SPRINGER-VERLAG, NEW YORK, vol. 42, no. 12, 15 September 2011 (2011-09-15), pages 3591-3601, XP019968016, ISSN: 1543-1940, DOI: 10.1007/S11661-011-0869-7
- Tata Steel Automotive: "DP800 CR High strength, high ductility, high formability", , 2013, XP002732812, Retrieved from the Internet: URL:http://www.tatasteelautomotive.com/sta tic_files/StaticFiles/Automotive/new-2013/ Tata%20Steel%20-%20DP800%20CR%20-%20data%2 0sheet.pdf [retrieved on 2014-11-21]
- SPEER J G ET AL: "Partitioning of carbon from supersaturated plates of ferrite, with application to steel processing and fundamentals of the bainite transformation", CURRENT OPINION IN SOLID STATE AND MATERIALS SCI, ELSEVIER SCIENCE LTD, OXFORD, GB, vol. 8, no. 3-4, 1 June 2004 (2004-06-01), pages 219-237, XP004742048, ISSN: 1359-0286, DOI: 10.1016/J.COSSMS.2004.09.003

## Description

### BACKGROUND

It is desirable to produce steels with high strength and good formability characteristics. However, commercial production of steels exhibiting such characteristics has been difficult due to factors such as the desirability of relatively low alloying additions and limitations on thermal processing capabilities of industrial production lines.

WO 2009/035576 A1 is directed to a method and apparatus of producing a dual-phase galvanized steel strip with improved formability while maintaining a high tensile strength. According to the disclosed process, the retained austenite is stabilized by bainite formation. The document does not disclose cooling of a steel that results in a transform of austenite to martensite.

EP2325346 (A1) discloses a high-strength steel alloys wherein the austenite content is in the range of 5% to 50%, and the proportion of the area of bainitic ferrite in upper bainite is 5% or more. Bainite formation is encouraged to stabilize retained austenite. The document does not disclose cooling of a steel that results in a transform of austenite to martensite.

EP2524970 (A1) discloses a method for manufacturing a high-strength flat steel product. In the disclosed method of producing the steel any coating process, such as hot dip coating processes, takes place after the heat treatment of the flat steel product is finished, i.e. after stabilizing austenite through a partitioning step. The document does not disclose a process comprising stabilizing austenite after hot dip coating of the steel sheet.

The present invention relates to processing methods for production of steel using hot-dip galvanizing/galvannealing (HDG) processes such that the resulting steel exhibits high strength and cold formability.

### SUMMARY

A modified HDG process for steel is provided that produces a resulting microstructure consisting of generally martensite and austenite (among other constituents). To achieve such a microstructure, the composition includes certain alloying additions and the HDG process includes certain process modification, all of which are at least partially related to driving the transformation of austenite to martensite followed by a partial stabilization of austenite at room-temperature.

The invention is defined by the appended claims.

### BRIEF DESCRIPTION OF THE FIGURES

The accompanying figures, which are incorporated in and constitute a part of this specification, illustrate embodiments, and together with the general description given above, and the detailed description of the embodiments given below, serve to explain the principles of the present disclosure.
FIGURE 1 depicts a schematic view of a HDG temperature profile with a partitioning step performed after galvanizing/galvannealing.
FIGURE 2 depicts a schematic view of a HDG temperature profile with a partitioning step performed during galvanizing/galvannealing.
FIGURE 3 depicts a plot of one embodiment with Rockwell hardness plotted against cooling rate.
FIGURE 4 depicts a plot of another embodiment with Rockwell hardness plotted against cooling rate.
FIGURE 5 depicts a plot of another embodiment with Rockwell hardness plotted against cooling rate.
FIGURE 6 depicts six photo micrographs of the embodiment of FIG. 3 taken from samples being cooled at various cooling rates.
FIGURE 7 depicts six photo micrographs of the embodiment of FIG. 4 taken from samples being cooled at various cooling rates.
FIGURE 8 depicts six photo micrographs of the embodiment of FIG. 5 taken from samples being cooled at various cooling rates.
FIGURE 9 depicts a plot of tensile data as a function of austenitization temperature for several embodiments.
FIGURE 10 depicts a plot of tensile data as a function of austenitization temperature for several embodiments.
FIGURE 11 depicts a plot of tensile data as a function of quench temperature for several embodiments.
FIGURE 12 depicts a plot of tensile data as a function of quench temperature for several embodiments.

### DETAILED DESCRIPTION

FIG. 1 shows a schematic representation of the thermal cycle used to achieve high strength and cold formability in a steel sheet having a certain chemical composition (described in greater detail below). In particular, FIG. 1 shows a typical hot-dip galvanizing or galvannealing thermal profile (10) with process modifications shown with dashed lines. In one embodiment the process generally involves austenitization followed by a rapid cooling to a specified quench temperature to partially transform austenite to martensite, and the holding at an elevated temperature, a partitioning temperature, to allow carbon to diffuse out of martensite and into the remaining austenite, thus, stabilizing the austenite at room temperature. In some embodiments, the thermal profile shown in FIG. 1 may be used with conventional continuous hot-dip galvanizing or galvannealing production lines, although such a production line is not required.

As can be seen in FIG. 1, the steel sheet is first heated to a peak metal temperature (12). The peak metal temperature (12) in the illustrated example is shown as being at least above the austenite transformation temperature (A₁) (e.g., the dual phase, austenite + ferrite region). Thus, at the peak metal temperature (12), at least a portion of the steel will be transformed to austenite. Although FIG. 1 shows the peak metal temperature (12) as being solely above A₁, it should be understood that in some embodiments the peak metal temperature may also include temperatures above the temperature at which ferrite completely transforms to austenite (A₃) (e.g., the single phase, austenite region).

Next the steel sheet undergoes rapid cooling. As the steel sheet is cooling, some embodiments may include a brief interruption in cooling for galvanizing or galvannealing. In embodiments where galvanizing is used, the steel sheet may briefly maintain a constant temperature (14) due to the heat from the molten zinc galvanizing bath. Yet in other embodiments, a galvannealing process may be used and the temperature of the steel sheet may be slightly raised to a galvannealing temperature (16) where the galvannealing process may be performed. According to further disclosed background art, the galvanizing or galvannealing process may be omitted entirely and the steel sheet may be continuously cooled.

The rapid cooling of the steel sheet is shown to continue below the martensite start temperature (M_{S}) for the steel sheet to a predetermined quench temperature (18). It should be understood that the cooling rate to Mₛ has to be high enough to transform at least some of the austenite formed at the peak metal temperature (12) to martensite. In other words the cooling rate must be rapid enough to transform austenite to martensite instead of other non-martensitic constituents such as ferrite, pearlite, or bainite which transform at relatively lower cooling rates.

As is shown in FIG. 1, the quench temperature (18) is below M. The difference between the quench temperature (18) and Mₛ may vary depending an the individual composition of the steel sheet being used. However, in many embodiments the difference between quench temperature (18) and Mₛ should be sufficiently great to form an adequate amount of martensite to act as a carbon source to stabilize the austenite and avoid creating excessive "fresh" martensite upon final cooling. Additionally, quench temperature (18) should be sufficiently high to avoid consuming too much austenite during the initial quench (e.g., to avoid excessive carbon enrichment of austenite greater than that required to stabilize austenite for the given embodiment).

In many embodiments, quench temperature (18) may vary from about 191 °C to about 281 °C, although no such limitation is required. Additionally, quench temperature (18) may be calculated for a given steel composition. For such a calculation, quench temperature (18) corresponds to the retained austenite having an Ms temperature of room temperature after partitioning. Methods for calculating quench temperature (18) are known in the art and described in J. G. Speer, A. M. Streicher, D. K. Matlock, F. Rizzo, and G. Krauss, "Quenching And Partitioning : A Fundamentally New Process to Create High Strength Trip Sheet Microstructures," Austenite Formation and Decomposition, pp. 505-522, 2003; and A. M. Streicher, J. G. J. Speer, D. K. Matlock, and B. C. De Cooman, "Quenching and Partitioning Response of a Si-Added TRIP Sheet Steel," in Proceedings of the International Conference on Advanced High Strength Sheet Steels for Automotive Applications, 2004.

The quench temperature (18) should be sufficiently low (with respect to Mₛ) to form an adequate amount of martensite to act as a carbon source to stabilize the austenite and avoid creating excessive "fresh" martensite upon the final quench. Alternatively, the quench temperature (18) should be sufficiently high to avoid consuming too much austenite during the initial quench and creating a situation where the potential carbon enrichment of the retained austenite is greater than that required for austenite stabilization at room temperature. In some embodiments, a suitable quench temperature (18) may correspond to the retained austenite having an Mₛ temperature of room temperature after partitioning. Speer and Streicher *et al.* (above) have provided calculations that provide guidelines to explore processing options that may result in desirable microstructures. Such calculations assume idealized full partitioning, and may be performed by applying the Koistinen-Marburger (KM) relationship twice (*fₘ* = 1 - *e*^{-1.1*x*10⁻²(Δ*T*))} - first to the initial quench to quench temperature (18) and then to the final quench at room temperature (as further described below). The Ms temperature in the KM expression can be estimated using empirical formulae based on austenite chemistry (such as that of the well known in the art Andrew's linear expression): $Ms \left(°C\right) = 539 - 423 C - 30.4 Mn - 7.5 Si + 30 Al$

The result of the calculations described by Speer et al. may indicate a quench temperature (18) which may lead to a maximum amount of retained austenite. For quench temperatures (18) above the temperature having a maximum amount of retained austenite, significant fractions of austenite are present after the initial quench; however, there is not enough martensite to act as a carbon source to stabilize this austenite. Therefore, for the higher quench temperatures, increasing amounts of fresh martensite form during the final quench. For quench temperatures below the temperature having a maximum amount of retained austenite, an unsatisfactory amount of austenite may be consumed during the initial quench and there may be an excess amount of carbon that may partition from the martensite.

Once the quench temperature (18) is reached, the temperature of the steel sheet is either increased relative to the quench temperature or maintained at the quench temperature for a given period of time. In particular, this stage may be referred to as the partitioning stage. In such a stage, the temperature of the steel sheet is at least maintained at the quench temperature to permit carbon diffusion from martensite formed during the rapid cooling and into any remaining austenite. Such diffusion permits the remaining austenite to be stable (or meta-stable) at room temperature, thus improving the mechanical properties of the steel sheet.

In some embodiments, the steel sheet may be heated above Mₛ to a relatively high partitioning temperature (20) and thereafter held at the high partitioning temperature (20). A variety of methods may be utilized to heat the steel sheet during this stage. By way of example only, the steel sheet may be heated using induction heating, torch heating, and/or the like. Alternatively, in other embodiments, the steel sheet may be heated but to a different, lower partitioning temperature (22) which is slightly below Mₛ. The steel sheet may then be likewise held at the lower partitioning temperate (22) for a certain period of time. In still a third alternative embodiment, another alternative partitioning temperature (24) may be used where the steel sheet is merely maintained at the quench temperature. Of course, any other suitable partitioning temperature may be used as will be apparent to those of ordinary skill in the art in view of the teachings herein.

After the steel sheet has reached the desired partitioning temperature (20, 22, 24), the steel sheet is maintained at the desired partitioning temperature (20, 22, 24) for a sufficient time to permit partitioning of carbon from martensite to austenite. The steel sheet may then be cooled to room temperature.

FIG. 2 shows an alternative further disclosed as background art of the thermal cycle described above with respect to FIG. 1 (with a typical galvanizing/galvannealing thermal cycle shown with a solid line (40) and departures from typical shown with a dashed line). In particular, like with the process of FIG. 1, the steel sheet is first heated to a peak metal temperature (42). The peak metal temperature (42) in the illustrated background art is shown as being at least above A₁. Thus, at the peak metal temperature (42), at least a portion of the steel sheet will be transformed to austenite. Of course, like the process of FIG. 1, this further disclosed background art may also include a peak metal temperature in excess of A3.

According to further disclosed background art, the steel sheet may next be rapidly quenched (44). It should be understood that the quench (44) may be rapid enough to initiate transformation of some of the austenite formed at the peak metal temperature (42) into martensite, thus avoiding excessive transformation to non-martensitic constituents such as ferrite, pearlite, banite, and/or the like.

According to further disclosed background art, quench (44) may be then ceased at a quench temperature (46). Like the process of FIG. 1, quench temperature (46) is below A. Of course, the amount below Ms may vary depending upon the material used. However, as described above, it is further disclosed as background art that the difference between quench temperature (46) and Ms may be sufficiently great to form an adequate amount of martensite yet be sufficiently low to avoid consuming too much austenite.

According to further disclosed background art, the steel sheet is then subsequently reheated (48) to a partitioning temperature (50, 52). Unlike the process of FIG. 1, the partitioning temperature (50, 52) according to the further disclosed as background art may be characterized by the galvanizing or galvannealing zinc bath temperature (if galvanizing or galvannealing is so used). For instance, it is further disclosed as background art that where galvanizing is used, the steel sheet may be re-heated to the galvanizing bath temperature (50) and subsequently held there for the duration of the galvanizing process. During the galvanizing process, partitioning may occur similar to the partitioning described above. Thus, the galvanizing bath temperature (50) may also function as the partitioning temperature (50). Likewise, where galvannealing is used according to the process of the background art further disclosed herein, the process may be substantially the same with the exception of a higher bath/partitioning temperature (52).

According to further disclosed background art, the steel sheet is further permitted to cool (54) to room temperature where at least some austenite may be stable (or meta-stable) from the partitioning step described above.

In some embodiments the steel sheet includes certain alloying additions to improve the propensity of the steel sheet to form a primarily austenitic and martensitic microstructure and/or to improve the mechanical properties of the steel sheet. Suitable compositions of the steel sheet include the following, by weight percent: 0.15-0.4% carbon, 1.5-4% manganese, 0-2% silicon or aluminum or some combination thereof, 0-0.5% molybdenum, 0-0.05% niobium, other incidental elements, and the balance being iron.

Further disclosed herein (but not claimed) are compositions of a steel including one or more of the following, by weight percent: 0.15-0.5% carbon, 1-3% manganese, 0-2% silicon or aluminum or some combination thereof, 0-0.5% molybdenum, 0-0.05% niobium, other incidental elements, and the balance being iron. Additionally, steel compositions of the further disclosed background art may include additions of vanadium and/or titanium in addition to, or in lieu of niobium, although such additions are entirely optional.

In the present invention carbon is used to stabilize austenite. For instance, increasing carbon may lower the Ms temperature, lower transformation temperatures for other non-martensitic constituents (e.g., bainite, ferrite, pearlite), and increase the time required for non-martensitic products to form. Additionally, carbon additions may improve the hardenability of the material thus retaining formation of non-martensitic constituents near the core of the material where cooling rates may be locally depressed. However, it should be understood that carbon additions may be limited as significant carbon additions may lead to detrimental effects on weldability.

Manganese provides additional stabilization of austenite by lowering transformation temperatures of other non-martensitic constituents, as described above. Manganese may further improve the propensity of the steel sheet to form a primarily austenitic and martensitic microstructure by increasing hardenability.

In other embodiments molybdenum may be used to increase hardenability.

In other embodiments silicon and/or aluminum may be provided to reduce the formation of carbides. It should be understood that a reduction in carbide formation may be desirable in some embodiments because the presence of carbides may decrease the levels of carbon available for diffusion into austenite. Thus, silicon and/or aluminum additions may be used to further stabilize austenite at room temperature.

According to further disclosed background art, nickel, copper, and chromium may be used to stabilize austenite. For instance, such elements may lead to a reduction in the Mₛ temperature. Additionally, nickel, copper, and chromium may further increase the hardenability of the steel sheet.

It is further disclosed herein that niobium may be used to increase the mechanical properties of the steel sheet. For instance, niobium may increase the strength of the steel sheet through grain boundary pinning resulting from carbide formation. According to a further disclosure other micro-alloying elements, such astitanium, vanadium, and/or the like may be used to increase the mechanical properties

In other embodiments, variations in the concentrations of elements and the particular elements selected may be made within the scope of the composition according to the claims. Of course, where such variations are made, it should be understood that such variations may have a desirable or undesirable effect an the steel sheet microstructure and/or mechanical properties in accordance with the properties described above for each given alloying addition.

### REFERENCE EXAMPLE 1

Reference examples of steel sheets were made with the compositions set forth in Table 1 below.

The materials were processed with a laboratory equipment according to the following parameters. Each sample was subjected to Gleeble 1500 treatments using copper cooled wedge grips and the pocket jaw fixture. Samples were austenitized at 1100°C and than cooled to room temperature at various cooling rates between 7-70°C/s.

**Table 1 Chemical compositions in weight %.**

| ID | Description | Al | C | Co | Cr | Cu | Mn | Mo | Nb | Ni | P | Si | Sn | Ti | V | W |
|---|---|---|---|---|---|---|---|---|---|---|---|---|---|---|---|---|
| V4037 | Lab Material | 1.41 | 0.19 | - | 0.01 | <0.003 | 1.54 | <0.003 | <0.003 | <0.003 | <0.003 | 0.11 | <0.003 | 0.01 | <0.003 | - |
| V4038 | Lab Material | 1.29 | 0.22 | - | 0.20 | <0.003 | 1.68 | <0.003 | 0.02 | <0.003 | 0.02 | 0.01 | <0.003 | 0.01 | <0.003 | - |
| V4039 | Lab Material | <0.003 | 0.20 | <0.002 | 0.01 | <0.002 | 2.94 | <0.002 | 0.00 | <0.002 | 0.00 | 1.57 | <0.002 | 0.01 | <0.002 | 0.00 |

### REFERENCE EXAMPLE 2

The Rockwell hardness of each of the steel compositions described in Example 1 and Table 1 above was taken an the surface of each sample. The results of the tests are plotted in FIGS. 3-5 with Rockwell hardness plotted as a function of cooling rate. The average of at least seven measurements is shown for each data point. The compositions V4037, V4038 and V4039 correspond to FIGS. 3, 4, and 5, respectively.

### REFERENCE EXAMPLE 3

Light optical micrographs were taken in the longitudinal through thickness direction near the center of each sample for each of the compositions of Example 1. The results of these tests are shown in FIGS. 6-8. The compositions V4037, V4038, and V4039 correspond to FIGS. 6, 7, and 8, respectively. Additionally, FIGS. 6-8 each contain six micrographs for each composition with each micrograph representing a sample subjected to a different cooling rate.

### REFERENCE EXAMPLE 4

A critical cooling rate for each of the compositions of Example 1 was estimated using the data of Examples 2 and 3 in accordance with the procedure described herein. The critical cooling rate herein refers to the cooling rate required to form martensite and minimize the formation of non-martensitic transformation products. The results of these tests are as follows:

| | |
|---|---|
| V4037: | 70 °C/s |
| V4038: | 75 °C/s |
| V4039: | 7 °C/s |

### EXAMPLE 5

Examples of steel sheets were made with the compositions set forth in Table 2 below.

The materials were processed by melting, hot rolling, and cold rolling. The materials were then subjected to testing described in greater detail below in Examples 6-7. All of the compositions listed in Table 2 were intended for use with the process described above with respect to FIG. 2 with the exception of invention example V4039 which was intended for use with the process described above with respect to FIG. 1. Heat V4039 had a composition intended to provide higher hardenability as required by the thermal profile described above with respect to FIG. 1. As a result V4039 was subjected to annealing at 600 °C for 2 hours in 100% H2 atmosphere after hot rolling, but prior to cold rolling. All materials were reduced during cold rolling about 75% to 1mm. Results for some of the material compositions set forth in Table 2 after hot rolling and cold rolling are shown in Tables 3 and 4, respectively.

**Table 2 Chemical compositions in weight %.**

| **Heat** | **Description** | **C** | **Mn** | **Si** | **Al** | **Mo** | **Cr** | **Nb** | **B** |
|---|---|---|---|---|---|---|---|---|---|
| V4037 | Lab Material | 0.19 | 1.54 | 0.11 | 1.41 | 0 | 0.009 | 0 | 0.0007 |
| V1307 | Lab Material | 0.19 | 1.53 | 1.48 | 0.041 | 0 | 0 | 0 | 0.0005 |
| V4063 | Lab Material | 0.19 | 1.6 | 0.11 | 1.34 | 0 | 0.003 | 0 | 0.0007 |
| V4038 | Lab Material | 0.22 | 1.68 | 0.007 | 1.29 | 0 | 0.2 | 0.021 | 0.0008 |
| V4039 | Lab Material | 0.2 | 2.94 | 1.57 | <0.030 | <0.002 | 0.005 | 0.002 | N/R |
| V1305 | Lab Material | 0.2 | 2.94 | 1.57 | 0 | 0 | 0 | 0 | 0.0006 |
| V4107 | Lab Material | 0.18 | 4.03 | 1.63 | 0.005 | 0 | 0 | 0 | 0.0008 |
| V4108 | Lab Material | 0.18 | 5.06 | 1.56 | 0.004 | 0 | 0 | 0 | 0.0009 |
| V4060 | Lab Material | 0.4 | 1.2 | 1.97 | 0.003 | 0 | 0.19 | 0.007 | 0.0005 |
| V4061 | Lab Material | 0.41 | 1.2 | 0.98 | 0.003 | 0 | 0.003 | 0 | 0.0004 |
| V4062 | Lab Material | 0.39 | 1.18 | 0.012 | 1.16 | 0 | 0.003 | 0 | 0.0007 |
| V4078-1 | Lab Material | 0.2 | 1.67 | 0.1 | 1.41 | 0.28 | 0.003 | <0.003 | 0.0007 |
| V4078-2 | Lab Material | 0.2 | 1.67 | 0.1 | 1.41 | 0.27 | <0.003 | 0.051 | 0.0007 |
| V4079-1 | Lab Material | 0.19 | 1.94 | 0.098 | 1.43 | <0.003 | <0.003 | <0.003 | 0.0007 |
| V4079-2 | Lab Material | 0.19 | 1.96 | 0.099 | 1.41 | <0.003 | <0.003 | 0.051 | 0.0007 |

**Table 3 - Tensile Data, Post Hot Rolling**

| **Heat** | **YPE (%)** | **Upper YS** | | **Lower YS** | | **Yield 0.2% Strength Offset** | | **UTS** | | **Total Elongation** | **Uniform Elongation** | **Hardness HRA** |
|---|---|---|---|---|---|---|---|---|---|---|---|---|
| | | **MPa** | **ksi** | **MPa** | **ksi** | **MPa** | **ksi** | **MPa** | **ksi** | **(2")** | **%** | |
| V4063 | 0 | N/A | N/A | N/A | N/A | 375 | 54 | 652 | 95 | 26 | 15 | 53 |
| | 0 | N/A | N/A | N/A | N/A | 380 | 55 | 648 | 94 | 26 | 15 | 53 |
| V4039* | 0 | N/A | N/A | N/A | N/A | 640 | 93 | 1085 | 157 | 14 | 9 | 67 |
| V4039* (annealed) | 0 | N/A | N/A | N/A | N/A | 603 | 88 | 748 | 109 | 20 | 10 | 61 |
| V4060 | 06 | 645 | 94 | 637 | 92 | 633 | 92 | 883 | 128 | 20 | 11 | 63 |
| | 0.5 | 610 | 89 | 605 | 88 | 611 | 89 | 876 | 127 | 22 | 12 | 61 |
| V4061 | 0 | N/A | N/A | N/A | 0 | 496 | 72 | 790 | 115 | 22 | 11 | 60 |
| | 0 | N/A | N/A | N/A | 0 | 507 | 74 | 799 | 116 | 20 | 11 | 60 |
| V4062 | 1.1 | 507 | 74 | 501 | 73 | 506 | 73 | 712 | 103 | 26 | 12 | 60 |
| | 0.7 | 505 | 73 | 502 | 73 | 502 | 73 | 713 | 103 | 24 | 12 | 57 |
| V4078-1 | 0.8 | 427 | 62 | 416 | 60 | 425 | 62 | 594 | 86 | 32 | 18 | 51 |
| V4078-2 | 0.6 | 525 | 76 | 519 | 75 | 525 | 76 | 685 | 99 | 21 | 15 | 56 |
| V4079-1 | 1.8 | 364 | 53 | 361 | 52 | 361 | 52 | 544 | 79 | 30 | 17 | 48 |
| V4079-2 | 1.2 | 497 | 72 | 481 | 70 | 489 | 71 | 639 | 93 | 24 | 13 | 52 |

| | | | | | | | | | | | | |
|---|---|---|---|---|---|---|---|---|---|---|---|---|
| *Tensile test performed in transverse direction for V4039 | | | | | | | | | | | | |

**Table 4 - Tensile Data, Post Cold Rolling**

| **Heat** | **Yield Strength 0.2% Offset** | | **UTS** | | **Total Elongation (2") %** | **Uniform Elongation %** | **Hardness HRA** |
|---|---|---|---|---|---|---|---|
| | **MPa** | **ksi** | **MPa** | **ksi** | | | |
| V4037 | 927 | 134 | 971 | 141 | 4.8 | 1.4 | 64 |
| V4063 | 1046 | 152 | 1101 | 160 | 2.4 | 1.3 | 65 |
| V4038 | 1001 | 145 | 1054 | 153 | 5.5 | 1.6 | 65 |
| V4039 | 1149 | 167 | 1216 | 176 | 4.4 | 1.5 | 68 |
| V4060 | 1266 | 184 | 1393 | 202 | 5.4 | 1.9 | 69 |
| V4061 | 1187 | 172 | 1279 | 186 | 4.3 | 1.7 | 68 |
| V4062 | 1111 | 161 | 1185 | 172 | 4.3 | 1.7 | 66 |
| V4078-1 | 1047 | 152 | 1105 | 160 | 3.6 | 1.4 | 65 |
| V4078-2 | 1154 | 167 | 1209 | 175 | 4.2 | 1.4 | 66 |
| V4079-1 | 932 | 135 | 975 | 141 | 4.6 | 1.4 | 64 |
| V4079-2 | 1034 | 150 | 1078 | 156 | 3.9 | 1.3 | 66 |

### EXAMPLE 7

The compositions of Example 5 were subjected to Gleeble dilatomety. Gleeble dilatomety was performed in vacuum using a 101.6x25.4x1 mm samples with a c-strain gauge measuring dilation in the 25.4 mm direction. Plots were generated of the resulting dilation vs. temperature. Line segments were fit to the dilatometric data and the point at which the dilatometric data deviated from linear behavior was taken as the transformation temperature of interest (e.g., A₁, A₃, Mₛ). The resulting transformation temperatures are tabulated in Table 5.

Gleeble methods were also used to measure a critical cooling rate for each of the compositions of Example 5. The first method utilized Gleeble dilatomety, as described above. The second method utilized measurements of Rockwell hardness. In particular, after samples were subjected to Gleeble testing at range of cooling rates, Rockwell hardness measurements were taken. Thus, Rockwell hardness measurements were taken for each material composition with a measurement of hardness for a range of cooling rates. A comparison was then made between the Rockwell hardness measurements of a given composition at each cooling rate. Rockwell hardness deviations of 2 points HRA were considered significant. The critical cooling rate to avoid non-martensitic transformation product was taken as the highest cooling rate for which the hardness was lower than 2 point HRA than the maximum hardness. The resulting critical cooling rates are also tabulated in Table 5 for some of the compositions listed in Example 5.

**Table 5 - Transformation Temperatures and Critical Cooling Rate from Gleeble Dilatomety**

| **Heat** | **A₁ (°C)** | **A₃ (°C)** | **Mₛ (°C)** | **Critical Cooling Rate (°C/s)** | |
|---|---|---|---|---|---|
| | | | | **Gleeble Dilatometry** | **Gleeble/Hardness** |
| V4037 | 737 | 970 | 469 | Inconclusive | 65 |
| V4063 | 720 | 975 | 425 | 70 | - |
| V4038 | 791 | 980 | 441 | - | 65 |
| V4039 | 750 | 874 | 394 | <10 | 6 |
| V4060 | 725 | 975 | 325 | 30 | - |
| V4061 | 675 | 900 | 325 | 40 | 55 |
| V4062 | 700 | 975 | 375 | 30 | - |
| V4078-1 | 750 | 925 | 450 | 40 | 55 |
| V4078-2 | 790 | 980 | 425 | 40 | - |
| V4079-1 | 800 | 1000 | 430 | 40 | - |
| V4079-2 | 750 | 990 | 425 | 40 | - |

### EXAMPLE 8

The compositions of Example 5 were used to calculate quench temperature and a theoretical maximum of retained austenite. The calculations were performed using the methods of *Speer et al.*, described above. The results of the calculations are tabulated below in Table 6 for some of the compositions listed in Example 5.

**Table 6 - Quench Temperature and Theoretical Maximum of Retained Austenite**

| **Heat** | **QT (°C)** | **f(γ) Theoretical Maximum** |
|---|---|---|
| V4037 | 281 | 0.15 |
| V4063 | 278 | 0.15 |
| V4038 | 270 | 0.18 |
| V4039 | 203 | 0.2 |
| V4060 | 191 | 0.35 |
| V4061 | 196 | 0.36 |
| V4062 | 237 | 0.31 |
| V4078-1 | 276 | 0.16 |
| V4078-2 | 276 | 0.16 |
| V4079-1 | 273 | 0.16 |
| V4079-2 | 272 | 0.16 |

### EXAMPLE 9

The samples of the compositions of Example 5 were subjected to the thermal profiles shown in FIGS. 1 and 2 with peak metal temperature and quench temperature varied between samples of a given composition. As described above, only composition V4039 was subjected to the thermal profile shown in FIG. 1, while all other compositions were subjected to the thermal cycle shown in FIG. 2. For each sample, tensile strength measurements were taken. The resulting tensile measurements are plotted in FIGS. 9-12. In particular, FIGS. 9-10 show tensile strength data plotted against austenitization temperature and FIGS. 11-12 show tensile strength data plotted against quench temperature. Additionally, where the thermal cycles were performed using Gleeble methods, such data points are denoted with "Gleeble." Similarly, where thermal cycles were performed using a salt bath, such data points are denoted with "salt."

Additionally, similar tensile measurements for each composition listed in Example 5 (where available) are tabulated in Table 7, shown below. Partitioning times and temperatures are shown for example only, in other embodiments the mechanisms (such as carbon partitioning and/or phase transformations) occur during non-isothermal heating and cooling to or from the stated partitioning temperature which may also contribute to final material properties.

**Table 7 - Tensile Data, Post Partitioning**

| **Heat** | **Peak Metal Temp [°C]** | **Quench Temp (°C)** | **Partitioning Temp (°C)** | **Partitioning Time(s)** | **0.2% Yield Strength** | **Ultimate Tensile Strength** | **Total Elongation (%)** | **TE x UTS (Mpa x %)** |
|---|---|---|---|---|---|---|---|---|
| V1307 | 800 | 250 | 466 | 30 | 419 | 818 | 27 | 22,424 |
| | 800 | 250 | 466 | 30 | 416 | 807 | 28 | 22,345 |
| | 850 | 250 | 466 | 30 | 553 | 862 | 25 | 21,805 |
| | 850 | 250 | 466 | 30 | 535 | 847 | 25 | 21,336 |
| | 900 | 250 | 466 | 30 | 548 | 854 | 24 | 20,144 |
| | 800 | 250 | 400 | 30 | 445 | 898 | 22 | 19,675 |
| | 900 | 250 | 466 | 30 | 566 | 856 | 23 | 19,594 |
| | 800 | 250 | 400 | 30 | 432 | 889 | 22 | 19,478 |
| V4060 | 800 | 160 | 466 | 15 | 746 | 1317 | 23 | 29,630 |
| | 800 | 200 | 466 | 15 | 716 | 1332 | 19 | 25,309 |
| | 800 | 250 | 466 | 15 | 718 | 1403 | 18 | 25,115 |
| | 800 | 200 | 466 | 15 | 632 | 1309 | 19 | 24,746 |
| | 800 | 250 | 466 | 15 | 701 | 1379 | 18 | 24,407 |
| | 800 | 160 | 466 | 15 | 845 | 1311 | 18 | 23,986 |
| | 850 | 250 | 466 | 15 | 891 | 1291 | 18 | 23,749 |
| | 850 | 250 | 466 | 15 | 735 | 1223 | 19 | 23,729 |
| V4037 | 850 | 300 | 466 | 15 | 443 | 657 | 32 | 20,763 |
| | 921 | 200 | 466 | 30 | 325 | 612 | 34 | 20,633 |
| | 850 | 250 | 466 | 15 | 405 | 696 | 30 | 20,543 |
| | 921 | 300 | 466 | 30 | 380 | 591 | 34 | 20,090 |
| | 921 | 356 | 466 | 30 | 386 | 592 | 34 | 20,078 |
| | 921 | 400 | 466 | 30 | 388 | 588 | 34 | 19,937 |
| | 940 | 200 | 466 | 30 | 362 | 598 | 33 | 19,906 |
| | 850 | 200 | 466 | 15 | 427 | 687 | 28 | 19,022 |
| | 940 | 200 | 466 | 30 | 353 | 592 | 32 | 18,989 |
| | 980 | 200 | 466 | 30 | 341 | 612 | 31 | 18,897 |
| | 900 | 300 | 466 | 15 | 493 | 727 | 26 | 18,767 |
| | 850 | 200 | 466 | 15 | 447 | 702 | 27 | 18,600 |
| | 850 | 300 | 466 | 15 | 404 | 678 | 27 | 18,435 |
| | 980 | 200 | 466 | 30 | 347 | 611 | 30 | 18,387 |
| | 940 | 200 | 466 | 30 | 330 | 548 | 33 | 18,253 |
| | 980 | 200 | 466 | 30 | 345 | 612 | 29 | 17,939 |
| V4038 | 850 | 300 | 466 | 15 | 481 | 754 | 26 | 19,536 |
| | 918 | 400 | 466 | 30 | 377 | 681 | 27 | 18,461 |
| | 918 | 286 | 466 | 30 | 357 | 695 | 26 | 18,348 |
| | 918 | 200 | 466 | 30 | 363 | 697 | 26 | 18,193 |
| | 918 | 300 | 466 | 30 | 354 | 696 | 26 | 17,949 |
| | 850 | 300 | 466 | 15 | 457 | 773 | 23 | 17,777 |
| V4039 | 800 | 250 | 400 | 60 | 821 | 1299 | 15 | 19,225 |
| | 800 | 250 | 400 | 60 | 821 | 1298 | 15 | 18,945 |
| | 900 | 250 | 400 | 60 | 923 | 1273 | 15 | 18,593 |
| | 850 | 250 | 400 | 60 | 874 | 1278 | 14 | 18,142 |
| | 900 | 250 | 400 | 60 | 913 | 1258 | 14 | 17,984 |
| V4060 | 800 | 160 | 466 | 15 | 746 | 1317 | 23 | 29,630 |
| | 800 | 200 | 466 | 15 | 716 | 1332 | 19 | 25,309 |
| | 800 | 250 | 466 | 15 | 718 | 1403 | 18 | 25,115 |
| | 800 | 200 | 466 | 15 | 632 | 1309 | 19 | 24,746 |
| | 800 | 250 | 466 | 15 | 701 | 1379 | 18 | 24,407 |
| | 800 | 160 | 466 | 15 | 845 | 1311 | 18 | 23,986 |
| | 850 | 250 | 466 | 15 | 891 | 1291 | 18 | 23,749 |
| | 850 | 250 | 466 | 15 | 735 | 1223 | 19 | 23,729 |
| | 800 | 200 | 466 | 30 | 942 | 1319 | 17 | 22,422 |
| | 850 | 200 | 466 | 15 | 695 | 1222 | 16 | 19,070 |
| V4061 | 750 | 250 | 466 | 15 | 553 | 985 | 20 | 19,902 |
| | 750 | 250 | 466 | 15 | 581 | 918 | 21 | 18,996 |
| V4062 | 750 | 200 | 466 | 15 | 478 | 813 | 23 | 18,778 |
| | 750 | 250 | 466 | 15 | 480 | 816 | 22 | 17,944 |
| | 750 | 200 | 466 | 15 | 536 | 790 | 23 | 17,936 |
| V4107 | 850 | 250 | 400 | 60 | 776 | 1382 | 13 | 17,824 |
| V4108 | 900 | 250 | 400 | 60 | 923 | 1642 | 11 | 17,401 |
| | 850 | 250 | 400 | 60 | 952 | 1620 | 11 | 17,337 |
| V4078-1 | 850 | 300 | 466 | 15 | 448 | 783 | 24 | 19,016 |
| | 850 | 300 | 466 | 15 | 492 | 761 | 24 | 17,888 |
| V4078-2 | 900 | 250 | 466 | 30 | 713 | 843 | 21 | 17,946 |
| | 850 | 300 | 466 | 15 | 689 | 859 | 20 | 17,525 |
| | 850 | 300 | 466 | 15 | 671 | 871 | 20 | 17,503 |

It will be understood various modifications may be reasonably made to this invention without departing from the scope of the claims. Therefore, the limits of this invention should be determined from the appended claims.

## Claims

1. A method for producing a hot dip galvanized/galvannealed steel sheet, the steel sheet consisting of the following elements by weight percent:
0.15-0.4% carbon;
1.5-4% manganese;
2% or less silicon, aluminum, or some combination thereof;
0.5% or less molybdenum;
0.05% or less niobium;
the balance being iron and other incidental impurities;
wherein the steel sheet has a microstructure consisting of generally martensite and austenite;
the method comprising the steps of
(a) heating the steel sheet to a first temperature T1, wherein T1 is at least above the temperature at which the steel sheet transforms to austenite and ferrite;
(b) cooling the steel sheet to a second temperature T2 which is sufficiently low with respect to the martensite start temperature Ms to form an adequate amount of martensite to act as a carbon source to stabilize the austenite and avoid creating excessive "fresh" martensite upon the final quench and which is sufficiently high to avoid consuming too much austenite during the initial quench by cooling at a cooling rate, wherein T2 is below the martensite start temperature Ms, wherein the cooling rate is sufficiently rapid to transform austenite to martensite and to avoid the formation of non-martensitic transformation products;
(c) subjecting the steel sheet to hot dip galvanizing or galvannealing while cooling the steel sheet to T2;
(d) re-heating the steel sheet to a partitioning temperature, wherein the partitioning temperature is sufficient to permit diffusion of carbon within the structure of the steel sheet;
(e) stabilizing austenite by holding the steel sheet at the partitioning temperature for a holding time, wherein the holding time is of a period of time sufficient to permit diffusion of carbon from martensite to austenite; and
(f) cooling the steel sheet to room temperature.

2. The method of claim 1, wherein the hot dip galvanizing or galvannealing occurs above Ms.

3. The method of claim 1, wherein the partitioning temperature is above Ms.

4. The method of claim I, wherein the partitioning temperature is below Ms.

## Patentansprüche

1. Verfahren zur Herstellung eines feuerverzinkten/galvannealten Stahlblechs, wobei das Stahlblech aus den folgenden Elementen nach Gewichtsprozenten besteht: 0,15 - 0,4 % Kohlenstoff;
1,5 - 4 % Mangan;
2 % oder weniger Silizium, Aluminium oder eine Kombination davon;
0,5 % oder weniger Molybdän;
0,05 % oder weniger Niob;
Rest Eisen oder andere übliche Verunreinigungen;
wobei das Stahlblech eine Mikrostruktur aufweist, welche im Wesentlichen aus Martensit und Austenit besteht;
wobei das Verfahren die Schritte umfasst:
(a) Erhitzen des Stahlblechs auf eine erste Temperatur T1, wobei T1 mindestens über der Temperatur liegt, bei welcher das Stahlblech zu Austenit und Ferrit transformiert;
(b) Abkühlen des Stahlblechs auf eine zweite Temperatur T2, welche in Bezug auf die Martensit-Starttemperatur Ms ausreichend niedrig ist, um eine ausreichende Menge Martensit zu bilden, um als Kohlenstoffquelle zu dienen, um das Austenit zu stabilisieren und die Bildung von überschüssigem "frischem" Martensit beim abschließenden Quenchen zu vermeiden, und welche ausreichend hoch ist, um den Verbrauch von zu viel Austenit während des initialen Quenchens durch Kühlen bei einer Kühlrate zu vermeiden, wobei T2 unter der Martensit-Starttemperatur Ms liegt, wobei die Kühlrate ausreichend schnell ist, um Austenit in Martensit zu transformieren und die Bildung von nicht-martensitischen Transformationsprodukten zu vermeiden;
(c) Unterziehen des Stahlblechs einer Feuerverzinkung oder Galvannealung während des Abkühlens des Stahlblechs auf T2;
(d) Wiedererhitzen des Stahlblechs auf eine Partitionierungstemperatur, wobei die Partitionierungstemperatur ausreichend ist, um eine Diffusion von Kohlenstoff innerhalb der Struktur des Stahlblechs zuzulassen;
(e) Stabilisieren von Austenits durch Halten des Stahlblechs bei einer Partitionierungstemperatur für eine Haltezeit, wobei die Haltezeit eine Zeitspanne ist, welche ausreichend ist, um Diffusion von Kohlenstoff von Martensit zu Austenit zuzulassen; und
(f) Kühlen des Stahlblechs auf Raumtemperatur.

2. Verfahren nach Anspruch 1, wobei Feuerverzinken oder Galvannealen oberhalb Ms erfolgt.

3. Verfahren nach Anspruch 1, wobei die Partitionierungstemperatur oberhalb von Ms ist.

4. Verfahren nach Anspruch 1, wobei die Partitionierungstemperatur unterhalb von Ms ist.

## Revendications

1. Procédé pour produire une tôle d'acier galvanisée par immersion à chaud / recuite par galvanisation, la tôle d'acier étant constituée des éléments suivants, en pourcentages en poids :
0,15 à 0,4 % de carbone ;
1,5 à 4 % de manganèse ;
2 % ou moins de silicium, d'aluminium, ou d'une de leurs combinaisons ;
0,5 % ou moins de molybdène ;
0,05 % ou moins de niobium ;
le reste étant du fer et d'autres impuretés accidentelles ;
dans lequel la tôle d'acier a une microstructure consistant généralement en martensite et austénite ; le procédé comprenant les étapes de
(a) chauffage de la tôle d'acier à une première température T1, laquelle T1 est au moins supérieure à la température à laquelle la tôle d'acier se transforme en austénite et ferrite ;
(b) refroidissement de la tôle d'acier à une deuxième température T2 qui est suffisamment basse par rapport à la température de début de martensite Ms pour former une quantité adéquate de martensite pour agir en tant que source de carbone pour stabiliser l'austénite et éviter la création de martensite "fraîche" excessive suite à la trempe finale et qui est suffisamment élevée pour éviter la consommation de trop d'austénite durant la trempe initiale par refroidissement à une certaine vitesse de refroidissement, laquelle T2 est inférieure à la température de début de martensite Ms, et laquelle vitesse de refroidissement est suffisamment élevée pour transformer l'austénite en martensite et pour éviter la formation de produits de transformation non martensitiques ;
(c) soumission de la tôle d'acier à une galvanisation par immersion à chaud ou recuite par galvanisation pendant le refroidissement de la tôle d'acier à T2 ;
(d) de nouveau chauffage de la tôle d'acier à une température de séparation, laquelle température de séparation est suffisante pour permettre la diffusion de carbone à l'intérieur de la structure de la tôle d'acier ;
(e) stabilisation de l'austénite par maintien de la tôle d'acier à la température de séparation pendant un certain temps de maintien, lequel temps de maintien est une période de temps suffisante pour permettre la diffusion de carbone de la martensite à l'austénite ; et
(f) refroidissement de la tôle d'acier à la température ambiante.

2. Procédé selon la revendication 1, dans lequel la galvanisation par immersion à chaud ou le recuit par galvanisation a lieu à une température supérieure à Ms.

3. Procédé selon la revendication 1, dans lequel la température de séparation est supérieure à Ms.

4. Procédé selon la revendication 1, dans lequel la température de séparation est inférieure à Ms.
